

## UNITED STATES PATENT OFFICE

2,040,927

## COLORATION OF TEXTILE MATERIALS

George Holland Ellis and Ernest William Kirk,  
Spondon, near Derby, England, assignors to  
Celanese Corporation of America, a corporation  
of Delaware

No Drawing. Application October 6, 1932, Serial  
No. 636,578. In Great Britain October 26,  
1931

15 Claims. (Cl. 8—6)

This invention relates to the coloration of textile materials and more particularly to the coloration of such materials by the so-called "azoic process" wherein insoluble or difficultly soluble

5 azo dyes are formed on the materials by the coupling thereon of diazo compounds and suitable coupling components.

The coloration of cellulosic materials by the azoic process has long been practised on an extensive scale and as an example may be mentioned the production of the well-known para-nitraniline red on cotton materials from diazotized para-nitraniline and  $\beta$ -naphthol. During the past decade the scope of the azoic process 10 has been very largely extended by the introduction of new coupling components, more particularly arylamides of 2:3-hydroxy-naphthoic acid and the diacetoacetyl derivatives of aromatic diamines, of which the diaceto-acetyl-ortho-tolidine is possibly the best known example. By 15 the use of these coupling components in conjunction with diazo compounds, especially those of the benzene and naphthalene series, a wide range of colorations has been produced, many of which exhibit outstanding properties of fastness, particularly to the action of light or the action 20 of hot alkaline or soap solutions. In this series of colors, however, there has in the past been a marked lack of blues and greens, the latter in 25 particular being practically non-existent.

We have found that diazotizable derivatives of 1:4-diamino anthraquinone or 1:4-amino-hydroxy anthraquinone constitute very valuable diazo components for the production of colorations on 30 textile materials by the azoic process. By employing these diazo components we have found it possible to produce bright blue and green shades which could hitherto only be obtained with great difficulty or not at all by azoic processes. Further, 35 these colorations so produced exhibit very good fastness properties, particularly in respect of fastness to hot soaping treatments. The latter is a point of particular importance in the case of yarns, particularly artificial yarns, which are to be woven with silk in the gummed state and so are called upon to resist the degumming treatment to which the resulting fabrics are necessarily subjected. For example, by coupling on 40 the material diazotized 1-amino-4-(4'-amino-phenylamino) anthraquinone with the meta-nitranilide of 2:3-hydroxy-naphthoic acid a full 45 bright blue shade may be produced, and by coupling with diaceto-acetyl-ortho-tolidine a bright bottle-green of desirable shade and good fastness properties. Again, by coupling the same diazo

component with an arylamide of an ortho hydroxy carboxylic acid of carbazole, full neutral grey shades may be produced having outstanding fastness properties.

Broadly, our invention comprises the coloration of textile materials by coupling thereon suitable coupling components with diazo compounds of diazotizable 1:4-diamino anthraquinone derivatives or 1:4-amino-hydroxy-anthraquinone derivatives. Preferably in the case of the 1:4-diamino 10 anthraquinone derivatives, neither of the 1:4-amino groups should be acylated and in the case of 1:4-amino hydroxy derivatives, the amino group should not be acylated nor should the hydroxy group be either acylated or etherified. 15

A wide range of diazotizable amino anthraquinone derivatives fulfilling the foregoing requirements is available, unsulphonated components being preferably employed. As examples of suitable diazo components may be mentioned the mono-aryl, mono-alkyl or mono-aralkyl derivatives of 1:4-diamino anthraquinone, whether the anthraquinone nucleus is further substituted or not. Of particular value are those anthraquinone compounds which may be diazotized so as to yield 20 diazo compounds containing in the 1:4-position two amino groups or one amino group and one hydroxy group, the amino group or groups not being acylated nor the hydroxy group acylated or etherified. Of this class of compounds, special 25 mention may be made of arylated 1:4-diamino or 1:4-amino-hydroxyanthraquinone derivatives containing in the aryl residue or residues one or more diazotizable amino groups. As examples of such compounds mention may be made of 1-amino- or 1-methylamino-4-(4'-amino-phenylamino) anthraquinone and 1-hydroxy-4-(4'-amino-phenylamino) anthraquinone. Other compounds may be employed, however, for example 30 1:4-diamino or 1:4-amino-hydroxy anthraquinones containing in a position other than the 1:4-position and especially in a hetero-nuclear position, a diazotizable amino group or a substituent, e. g. an arylamino, arylhydroxy, or aracylamino group containing a diazotizable amino group. An 35 example of such a compound is, for instance, 1:5-diamino-4-phenylamino anthraquinone.

Any desired coupling components may be utilized for the formation of dyestuffs by reaction 40 with the foregoing diazo components, for example amines or phenols, whether of the benzene, naphthalene or other series, and compounds containing methylene groups capable of reacting with diazo compounds, for example pyrazolone derivatives or acyl-acetic esters or acyl-acetic amides 45 50 55

or substituted amides, or other  $\beta$ -keto-acidyl compounds.

Particular mention may, however, be made of those coupling components capable of yielding 5 with diazo compounds azo dyestuffs of very difficultly soluble character and having little or no affinity for textile materials, whether natural or artificial, when applied thereto in substance. Examples of such coupling components are the 10 acylamino coupling components referred to in British Patent No. 404,363, and other amides and substituted amides, particularly arylamides, of hydroxy carboxylic acids, especially ortho-hydroxy carboxylic acids, of the benzene, naphthalene, carbazole and other series. Mention may 15 be made, for instance, of the anilides and naphthalides and substituted anilides or naphthalides of salicylic acid and its homologues, or of 2:3- or 1:4-hydroxy naphthoic acid, for example 2:3- 20 oxy naphthoic-ortho-toluide or meta-nitranilide. Compounds containing more than one hydroxy carboxylic acid residue may also be used, for instance the di(2:3-hydroxy-naphthoyl) dianisidine. Another class of coupling component yielding 25 difficultly soluble dyestuffs, and in consequence shades of excellent fastness, is the class of di- $\beta$ -keto-acidyl derivatives of aromatic diamines, for example the diaceto-acetyl derivative of orthotolidine or other aromatic diamine.

30 As regards the shades obtainable in accordance with the invention, it is found that, in general, blue to violet shades are obtained with those coupling components which normally yield orange to red shades with simple diazo compounds of the 35 benzene series, as for example 2:3-hydroxy-naphthoic anilide or meta-nitranilide. With those coupling components however which normally yield yellow shades with simple diazo compounds, green shades are in general obtained, as 40 is the case for instance when diaceto-acetyl ortho-tolidine is coupled with one of the special diazo components of the present invention, especially one of those which may be diazotized so as to obtain a diazo compound still containing 45 the 1:4-diamino- or 1:4-amino-hydroxy- grouping. Still other shades, some of great value, may however be obtained. Thus, with the arylamides of hydroxy carbazole carboxylic acids and the special anthraquinone diazo components, grey 50 shades of good fastness properties may be obtained.

As previously indicated, the diazo components employed in accordance with the present invention include diazotizable 1:4-diamino or 1:4-amino-hydroxyanthraquinone derivatives containing amino groups external to the anthraquinone nucleus, for example in an aryl residue linked to the anthraquinone residue. These new diazo components possess advantages not only in respect 55 of the shades obtained thereby, but also as regards the relative ease with which they may be diazotized as compared with those compounds in which an amino group is directly linked to an anthraquinone residue. We have, in fact, found 60 that anthraquinone derivatives in general containing "external" diazotizable amino groups constitute valuable diazo components for use in the production of azo dyes, whether in substance or on textile material or other substrata. As examples 65 may be mentioned for instance, in addition to the amino-aryl derivatives of 1:4-diamino- or 1:4-amino-hydroxy-anthraquinone above mentioned, aracylated derivatives of 1:4-diamino- or 1:4-amino-hydroxyanthraquinones sub-

stituted in the aracyl residue by amino groups. Compounds other than those derived from 1:4-diamino or 1:4-amino-hydroxy-anthraquinones may, however, also be used, for instance amino aracyl derivatives of other amino anthraquinones, for instance 1-amino- or 1:5- or 1:8-diamino anthraquinone, or amino aryl derivatives of these amino anthraquinones, for instance 1:5-di(para-amino-phenylamino) - anthraquinone or 1-(para-amino-phenylamino) - anthraquinone or 1-amino- 5-(para-amino-phenylamino) -anthraquinone.

In coloring textile materials in accordance with the new azoic process, any desired mode of working may be adopted. Thus the materials impregnated with the coupling components may be treated with solutions of the diazo compounds. Again, the diazo component may be applied first, diazotized on the material and the latter thereafter subjected to the action of the coupling component. Another method of operation consists in applying both the diazo component and the coupling component to the materials, either together or separately, and thereafter subjecting the materials to treatment adapted to effect diazotization of the diazo component and coupling with the coupling component.

Where the diazo component contains both a nuclear diazotizable amino group and an "external" diazotizable amino group, the latter may generally be preferentially diazotized leaving the other intact. Such preferential diazotization often leads to valuable results and may be effected, for instance, by diazotizing with sodium nitrite in the presence of a weak acid, e. g. an organic acid such as acetic acid. For example, by applying 1-amino-4-p-amino-phenylamino-anthraquinone to cellulose acetate, diazotizing with acetic acid and sodium nitrite and coupling with phenol, a green shade is obtained, whereas if the base is tetrazotized by using sodium nitrite and hydrochloric acid a brown shade is obtained.

The new processes may be utilized either for the uniform or for the local coloration of materials. In the former case the components may be applied by dyeing methods, or, if desired, by mechanical impregnation, for instance by padding or by all-over printing. For the production of local colorations, printing, stencilling or any other desired means may be employed, whether the components are applied together or separately or whether diazotization is effected on the material or in a separate operation.

The particular method to be used and the details to be observed in any given case in order to secure the best results depend upon the character of the material to be colored. In the case of cotton or other cellulosic materials, for instance regenerated cellulose artificial silk, it is in general most convenient to apply first the coupling component in the form of an alkali metal salt, for instance by a padding treatment. The impregnated material is thereafter developed in a solution of the desired diazo compound, or such a solution, if necessary suitably thickened, applied by printing or other mode of local application, where localized color effects are required.

In the case of cellulose acetate or other cellulose ester or ether materials, it is in general found most advantageous to apply coupling components in the free state, for instance in the manner described in U. S. Patent No. 1,844,350 in the case of arylamides of hydroxynaphthoic acids, or in the manner described in U. S. Patent No. 1,986,883, in the case of aceto-acetic arylide cou-

pling components. In general the most satisfactory method, both from the point of view of the results obtained and from the point of view of simplicity, is to apply the diazo component and coupling component simultaneously in the form of aqueous dispersions, the diazotization and coupling being subsequently effected by treatment first in a bath containing sodium nitrite and acetic or other acid followed by treatment 10 with a weakly alkaline solution.

The dispersions of the diazo or coupling components may be obtained by any desired method, for example by fine milling or grinding with or without the aid of dispersors and/or protective 15 colloids, by precipitation in the presence of protective colloids, or by a simple treatment with dispersors, as described for instance in any of U. S. Patents Nos. 1,618,413, 1,618,414, 1,694,413, 1,690,481, 1,803,008, 1,840,572, 1,716,721, 1,928,- 20 647, 1,959,352 and 390,424 filed 4th September, 1929. In some cases the dispersion of the coupling component may be facilitated by the presence of small quantities of alkali.

In treating cellulose ester and ether materials 25 the absorption of either or both components may be facilitated if desired by incorporating swelling agents in the dyeing or padding liquors or printing pastes employed, or the materials may be pretreated with swelling agents. Alcohol is 30 particularly suitable for this purpose, though other swelling agents may be employed if desired.

The following table shows a few of the numerous shades obtainable on cellulose acetate in accordance with the invention:—

35

|    | Amine                                                    | Developer                      | Shade on cellulose acetate                          |    |
|----|----------------------------------------------------------|--------------------------------|-----------------------------------------------------|----|
| 40 | 1. 1-amino-4-para-tolyl-aminoanthraquinone.....          | Naphthol AS/BS.....            | Full violet                                         |    |
|    | 2. Do.....                                               | Do. AS/G.....                  | Sage green                                          |    |
|    | 3. 1-amino-4-para-anisylamino-anthraquinone.....         | Do. AS/BS.....                 | Blinish violet                                      |    |
|    | 4. Do.....                                               | Do. AS/G.....                  | Sage green rather brighter than No. 2               | 40 |
|    | 5. 1-amino-4-(3'-aminophenylamino) anthraquinone.        | Do. AS/BS.....                 | Full bluish violet                                  |    |
|    | 6. Do.....                                               | Do. AS/G.....                  | Full sage green                                     |    |
|    | 7. 1-amino-4-(4'-amino) phenylaminoanthraquinone.        | Do. AS/BS.....                 | Full bright blue                                    |    |
| 45 | 8. Do.....                                               | Do. AS/OL.....                 | Full brilliant blue slightly redder than preceding  | 45 |
|    | 9. Do.....                                               | Do. AS/LT.....                 | Bright blue                                         |    |
|    | 10. Do.....                                              | Do. AS/D.....                  | Full, slightly greener blue                         |    |
|    | 11. 1-amino-4-(4'-amino) phenylaminoanthraquinone        | Do. AS/LB.....                 | Full neutral grey                                   |    |
|    | 12. Do.....                                              | Do. AS/G.....                  | Full bright bottle green                            |    |
| 50 | 13. 1,5 diaminio-4,8-diphenylaminoanthraquinone.         | Do. AS/BS.....                 | Grey-violet                                         | 50 |
|    | 14. Do.....                                              | Do. AS/G.....                  | Yellowish sage                                      |    |
|    | 15. 1-oxy-4-(4'-amino phenylamino) anthraquinones        | Do. AS/D.....                  | Bright full blue, deeper and redder than No. 10     |    |
|    | 16. Do.....                                              | Do. AS/G.....                  | Full green slightly brighter and deeper than No. 12 |    |
|    | 17. Do.....                                              | Do. AS/LB.....                 | Brownish grey                                       |    |
| 55 | 18. 1-amino-4-p. tolylaminio anthraquinone.....          | Phenol.....                    | Puce                                                |    |
|    | 19. Do.....                                              | Phenyl-methyl pyrazolone.....  | Olive                                               | 55 |
|    | 20. Do.....                                              | Meta-phenylene-diamine.....    | Deep yellowish olive                                |    |
|    | 21. Do.....                                              | Beta-naphthol.....             | Violet                                              |    |
|    | 22. Do.....                                              | Betahydroxynaphthoic acid..... | Do.                                                 |    |
|    | 23. 1-amino-4-(4'-amino) phenylaminoanthraquinone        | Phenol.....                    | Fairly bright bottle green                          |    |
|    | 24. Do.....                                              | Phenol-methylpyrazolone.....   | Very deep bottle green                              |    |
| 60 | 25. Do.....                                              | Meta-phenylenediamine.....     | Very deep yellowish bottle green                    | 60 |
|    | 26. Do.....                                              | Beta-naphthol.....             | Blackish violet                                     |    |
|    | 27. Do.....                                              | Betahydroxynaphthoic acid..... | Bright reddish blue                                 |    |
|    | 28. 1-methyleamino-4-(4'-amino) phenylaminoanthraquinone | Phenol.....                    | Bright, clear green                                 |    |
|    | 29. 1-amino-4-phenylamino-5-hydroxyanthraquinone         | Resorcin.....                  | Brownish-grey                                       |    |
| 65 | 30. Do.....                                              | Metahydroxy diphenylamine..... | Nigger brown                                        | 65 |
|    | 31. 1-amino-4-phenylamino-anthraquinone.....             | Do. Naphthol AS/LB.....        | Do.                                                 | 70 |
|    | 32. Do.....                                              | Do. AS.....                    | Chocolate brown                                     |    |
|    | 33. 1-amino-4-methoxyanthraquinone.....                  | Do. AS/LB.....                 | Deep brick red                                      |    |
|    | 34. 1-amino-4-acetaminoanthraquinone.....                |                                | Khaki                                               |    |

70 As will be appreciated from the foregoing description, this invention is of especial value in connection with the coloration of cellulose ester and ether materials. In addition to cellulose acetate the invention may be applied to cellulose

formate, propionate or butyrate or ethyl or benzyl cellulose materials. Other materials may also be colored by the new process, for instance wool, silk and other animal fibres, also mixed materials of all kinds, for instance materials containing both animal and vegetable fibres or materials containing cellulose acetate or other artificial fibres in conjunction with cotton or other natural fibres. In the case of animal fibres the coupling components are preferably applied from very weakly alkaline baths, or even in the form of dispersions of the free compounds; in fact the methods specified as suitable for the treatment of cellulose ester and ether materials may in general be applied with satisfaction for the coloration of animal fibres.

The dyestuffs obtainable in accordance with the invention may also be produced in substance and in this form, especially when unsulphonated, constitute valuable pigment colors or dyestuffs 20 which may be used for direct coloration of cellulose ester or ether materials. Of particular value are those coloring matters obtainable from the diazo compounds which contain intact the 1:4-diamino or 1:4-amino-hydroxy grouping and especially 1-hydroxy-, 1-amino-, or 1-aliphatically substituted amino-4-arylaminio-anthraquinones containing a diazo group in the aryl residue. For instance, 1-methylamino-, 1-dimethylamino-, 1-hydroxyethylamino or other 1-hydroxy-alkyl-amino-4-(amino-arylaminio)-anthraquinone may be employed.

As coupling components, amines, phenols or keto-methylene compounds of relatively low mo-

lecular weight are advantageous, for example, amines or phenols, particularly monohydric phenols, of the benzene series, acylacetic arylides or pyrazolones. Thus by diazotizing 1-methylamino - 4 - p - aminophenylamino-anthraquinone 75

*Example II*

and coupling with phenol a dyestuff which dyes cellulose acetate directly in fast bright green shades is obtained.

Other coupling components which may be employed are, for instance, ortho- or meta-cresol, m-phenylene-diamine, m-aminophenol, dimethyl-aniline, m-hydroxy-diphenylamine, 1-phenyl-3-methyl-5-pyrazolone, and acetoacetic anilide or other acetoacetic arylide of the benzene series.

Where as in the case of 1-amino-4-amino-aryl-amino-anthraquinones the diazo component contains both a diazotizable amino group in the anthraquinone nucleus and an "external" diazotizable amino group, one or both may be diazotized and coupled. By effecting diazotization with a nitrite and a weak acid, for example acetic or other organic acid, the "external" amino group only may be diazotized. This procedure in general gives rise to dyestuffs of greater value, both as regards color and as regards affinity for cellulose esters or ethers, than when both amino groups are diazotized and coupled.

The new dyestuffs are conveniently applied to cellulose esters or ethers in the form for example of aqueous suspensions or dispersions. The latter may be prepared in any desired manner, for example by grinding or milling with or without dispersors and/or protective colloids, by dissolving in a solvent and pouring into water or by treatment with dispersors as described for instance in any of U. S. Patents Nos. 1,618,413, 1,618,414, 1,694,413, 1,690,481, 1,803,008, 1,840,572, 1,716,721, 1,928,647 and 1,959,352. Liquid, paste, powder or other preparation comprising the new dyestuffs, together with dispersors and/or protective colloids, comprise an important feature of the invention. Such preparations may be of a strength suitable for coloring purposes or, if desired, in more concentrated form adapted to yield dye baths, printing pastes or the like by dilution with water, with or without additional protective colloids and/or dispersing agents.

The following examples illustrate the invention, but are not to be considered as limiting it in any way:—

*Example I*

To dye 10 kilogrammes of cellulose acetate yarn a bright grass-green shade resistant to the conditions necessary for the degumming of silk, 100 grammes of 1-amino-4-(4'-amino)phenyl-amino anthraquinone and 60 grammes of diacetoacetyl-o-tolidine are dispersed by fine grinding and boiling with 500 grammes of Turkey red oil. This is then stirred into a dye bath containing 300 litres of soft water containing half a gramme of Marseilles soap per litre. The yarn is entered cold, and turned for one hour, the temperature during this period being raised to 70° C. The yarn is continually turned at this temperature until the required depth of shade is obtained, when it is lifted, rinsed, and entered into a cold bath containing 300 litre of 4 grammes per litre solution of sodium nitrite, acidified with 8 grammes per litre glacial acetic acid. After turning in this bath for half an hour, the yarn is again lifted and rinsed and entered cold into a developing bath containing two grammes per litre Marseilles soap and half a gramme per litre of sodium carbonate. It is worked in this bath for half an hour cold, then heated gradually to 75° C. and kept at this for half an hour. The yarn is then lifted, thoroughly rinsed, and dried or otherwise treated.

To dye 10 kilogrammes of cellulose acetate woven fabric a full bright green shade of good fastness to light and water, 100 grammes of 1-methylamino-4-(4'-amino)phenylamino-anthraquinone are dispersed with Turkey red oil and the fabric dyed with this dispersion in the usual manner. The fabric is then rinsed, and the color diazotized by running for half an hour in a diazotizing bath of the constitution described in Example I, then rinsed and entered into a bath containing 50 grammes of phenol, and worked in this for half an hour. Soda ash and soap are then added to make the bath concentration 1 and 2 grammes per litre respectively, and the temperature raised to 75° C. and the fabric worked at this temperature for half an hour, then rinsed off well, and dried or otherwise treated.

*Example III*

To dye 10 kilogrammes of cellulose acetate yarn a full nigger-brown of good fastness to water, 100 grammes of 1-amino-4-paratolylamino - 5 - hydroxy-anthraquinone are dispersed by boiling with 300 grammes of Turkey red oil and diluting with about 10 litres of hot soft water, and added to a dye-bath of 300 litres of soft water. The yarn is entered and worked in this bath for two hours during the first 1/2 hour the temperature being raised to 70° C. and maintained at this temperature for the remainder of the dyeing period. The yarn is then lifted and entered into a diazotizing bath containing 6 grammes per litre sodium nitrite and 12 cc. per litre of hydrochloric acid 30° Tw. and turned in this bath for half an hour at 25° C. After rinsing, the yarn is entered cold into 300 litres of soft water to which has been added 100 grammes of metahydroxy-diphenylamine previously dissolved in boiling water. The 40 yarn is worked in this bath for half an hour cold, 150 grammes of soap added and the temperature then raised gradually to 75° C. The yarn is turned at 75° C. for half an hour, and then soaped for a further half hour in a fresh soap bath of 45 similar length and concentration, and is finally lifted, rinsed and dried or otherwise treated.

*Example IV*

To dye 10 kilogrammes of cellulose acetate knit fabric a full blue of good fastness to washing, 50 grammes of 1-amino-4-(4'-amino)phenylamino-anthraquinone are dispersed as above, and 50 grammes of the ortho toluidide of beta-hydroxy-naphthoic acid are dissolved in 2 litres of water containing 10 grammes of caustic soda. These ingredients are then added to a dyebath of 250 litres to which has previously been added 100 grammes of good textile soap and 20 grammes of glucose. The fabric is entered at 50° C. and the temperature raised over half an hour to 75° C. and kept at this until the desired depth of base has been attained. The fabric is then lifted and entered into a diazotizing bath containing 4 65 grammes per litre sodium nitrite and 8 grammes per litre glacial acetic acid and worked in this bath for half an hour cold, again rinsed and then entered into a bath containing 1 gram per litre sodium carbonate and 5 grammes per litre soap. 70 After working in this bath for half an hour cold, the temperature is raised slowly to 75° C. and kept at this for half an hour. The fabric is then lifted, rinsed and dried, or otherwise treated as requisite.

*Example V*

To print cellulose acetate fabric a fast deep grey shade, the printing paste is made up as follows:—

|                                                             | Parts |
|-------------------------------------------------------------|-------|
| 5 2-hydroxy carbazole - 3 - carboxylic anilide—             | 30    |
| 10% paste—                                                  | 30    |
| 1 - amino - 4 - (4' - amino) phenylaminoanthra-<br>quinone— | 30    |
| 10 Methylated spirits—                                      | 10    |
| Gum arabic thickening 1:1—                                  | 30    |

The fabric is printed with a suitably engraved roller, dried, steamed for half an hour at a pressure of 5 lbs. to the square inch, washed off well and diazotized by treatment in a bath containing 4 grammes per litre of sodium nitrite and 8 cc. per litre of glacial acetic acid. The fabric is then washed off well, and soaped in a bath containing 1 gramme per litre sodium carbonate, and 20 2 grammes per litre soap, first in the cold and then for half an hour at 75° C. finally being rinsed and dried or otherwise treated as desired.

*Example VI*

25 To 34.3 grammes of 1-methylamino-4-p-amino-phenylaminoanthraquinone in the form of a finely divided suspension in 3 litres of cold water are added 7.2 grammes of sodium nitrite suitably dissolved in water, followed by 30 grammes of glacial acetic acid. The whole is then stirred for 4 hours, after which 10 grammes of phenol in 500 cc. water are added, and a 10% solution of soda ash then run in slowly with stirring till the liquors react alkaline. After further stirring the dyestuff is 35 filtered off and washed well, being retained preferably as an aqueous paste.

Applied to cellulose acetate fibres by dispersion methods, it yields bright green shades of excellent fastness properties.

40 What we claim and desire to secure by Letters Patent is:

1. Process for the coloration of textile materials which comprises coupling thereon an azo coupling component which couples in an aryl residue with a diazo compound obtainable by diazotizing an anthraquinone compound containing an external diazotizable amino group.

2. Process for the coloration of textile materials which comprises coupling thereon an azo coupling component which couples in an aryl residue with a diazo compound obtainable by diazotizing a 4 - (amino - arylamino) - anthraquinone having in the 1-position a substituent N.R<sub>1</sub>R<sub>2</sub>, wherein R<sub>1</sub> and R<sub>2</sub> represent hydrogen or alkyl.

55 3. Process for the coloration of textile materials which comprises coupling thereon an arylamide of an aromatic hydroxy carboxylic acid with a diazo compound obtainable by diazotizing an anthraquinone compound containing an external diazotizable amino group.

4. Process for the coloration of textile materials which comprises coupling thereon an arylamide of an aromatic hydroxy carboxylic acid 60 with a diazo compound obtainable by diazotizing an anthraquinone compound containing amino groups free from acetyl substituents in the 1-4-positions, said compound having a diazotizable amino group as a substituent in an arylamino group.

70 5. Process for the coloration of textile materials which comprises coupling thereon an arylamide of an aromatic hydroxy carboxylic acid with a diazo compound obtainable by diazotizing a 4-(amino-arylarnino)-anthraquinone having in

the 1-position a substituent N.R<sub>1</sub>R<sub>2</sub>, wherein R<sub>1</sub> and R<sub>2</sub> represent hydrogen or alkyl.

6. Process for the coloration of textile materials which comprises coupling thereon an arylamide of an aromatic hydroxy carboxylic acid 5 with a diazo compound obtainable by diazotizing a 1-amino-4-(4'-amino-phenylamino)-anthraquinone.

7. Process for the coloration of textile materials which comprises coupling thereon an arylamide of 2:3-oxy-naphthoic acid with a diazo compound obtainable by diazotizing an anthraquinone compound containing an external diazotizable amino group.

8. The process comprising coloring organic derivatives of cellulose by means of azo dyestuffs obtainable by coupling azo coupling components with diazo compounds obtainable by diazotizing anthraquinone compounds containing external diazotizable amino groups.

9. Process for the coloration of organic derivatives of cellulose which comprises coupling thereon an azo coupling component with a diazo compound obtainable by diazotizing an anthraquinone compound containing an external diazotizable amino group.

10. Process for the coloration of cellulose acetate which comprises coupling thereon a phenol of the benzene series with a diazotized 4-(amino-arylarnino)-anthraquinone having in the 1-position a substituent N.R<sub>1</sub>R<sub>2</sub>, wherein R<sub>1</sub> and R<sub>2</sub> represent hydrogen or alkyl.

11. Organic derivatives of cellulose colored by means of azo dyestuffs obtainable by coupling 35 azo coupling components with diazo compounds obtainable by diazotizing anthraquinone compounds containing external diazotizable amino groups.

12. Cellulose acetate materials colored by means of azo dyestuffs obtainable by coupling azo coupling components with diazo compounds obtainable by diazotizing anthraquinone compounds containing external diazotizable amino 45 groups.

## 13. An azo dyestuff of the formula



in which X is an anthraquinone radical wherein the group



in which R<sub>1</sub> and R<sub>2</sub> represent hydrogen or alkyl group, is in the 1-position and the —NH— group in the 4-position, Y is an aryl radical, and Z the residue of a coupling component consisting of an arylamide of an aromatic hydroxy carboxylic acid.

14. Process for the coloration of textile materials, which comprises coupling thereon an azo coupling component with a diazo compound obtainable by diazotizing a 1:4-amino-hydroxy-anthraquinone containing an external diazotizable amino group.

## 15. An azo dyestuff of the formula



in which X is an anthraquinone radical wherein  
the group



in which R<sub>1</sub> and R<sub>2</sub> represent hydrogen or alkyl

group, is in the 1-position and the —NH— group  
in the 4-position, Y is an aryl radical, and Z  
the residue of a coupling component which  
couples in an aryl residue with a diazo compound.

5  
GEORGE HOLLAND ELLIS.  
ERNEST WILLIAM KIRK.